

## UNITED STATES PATENT OFFICE

2,545,450

## RESIN TREATMENT OF WOOL FABRIC

John N. Dalton and William B. Kaupin, Lawrence, Mass., assignors to Pacific Mills, Lawrence, Mass., a corporation of Massachusetts

No Drawing. Application February 18, 1948,  
Serial No. 9,346

6 Claims. (Cl. 117—103)

1

The present invention relates to the treatment of wool or part wool textile fabrics and to the resulting textile fabrics. An object is to produce such a fabric retaining substantially the soft hand, tensile strength and resistance to wear of the fabric before treatment and with a durable resistance to shrinkage when laundered. Another object is to fix acid dyes in such a fabric. Another object is to provide a continuous process for such treatment.

Although numerous processes have been suggested to produce a wool fabric having a reduced tendency to shrink when laundered, the resulting fabrics have lacked, in whole or in part, some of those characteristics which are required for a satisfactory commercial wool fabric, principally the softness and flexibility, namely the soft feel and hand, of the untreated fabric.

In the practice of our invention we impregnate and swell a wool, or part wool, textile fabric with an aqueous solution or dispersion of certain resin-forming materials and an acid catalyst, and, after squeezing out excess liquid, we heat the wet fabric throughout from surface to surface homogeneously and so rapidly that the resin-forming materials on the wool practically instantaneously become so viscous that they have no time to migrate appreciably and do not so migrate and the resin distribution remains in effect homogeneous throughout the fabric from surface to surface. This we carry out by infra-red or radio frequency radiation by which we accomplish this homogeneous practically instantaneous heating of the wet fabric at between 140° and about 212° F. We thereby prohibit the concentration of resin at or near the surfaces of the fabric which we have found to be a cause of the harsh finish of wool fabrics as previously treated with resin and we obtain a resin treated fabric which is homogeneous from surface to surface.

We then condense or polymerize the resin-forming material with the wool of the fabric to a water-insoluble condition by heating the fabric and at the same time retaining the resin-forming material evenly and uniformly distributed throughout the fabric and without migration of the resin-forming material to the surfaces of the fabric. The heating may be carried out by any suitable apparatus. We prefer to use the radiation of infra-red lamps. The temperature of the cloth may be raised to from 180° to 300° F. without causing migration of the resin-forming material and without impairing the flexibility and softness of the fabric and the resin contained therein.

2

The finished fabric has the softness, flexibility, tensile strength and wear resistance of the untreated fabric and has the desired improvement in dimensional stability, i. e., resistance to shrinkage on repeated laundering. It has an enhanced fixation of acid dyes.

The resin-forming materials in the impregnating bath may be either in the monomeric state or may be partially condensed to a low-molecular-weight reaction product which is capable of being dissolved or dispersed in water. By "solution" as used herein we include such dispersions. The resin-forming materials which we employ are the methylolmelamines including the alkylated methylolmelamines and preferably in addition thereto urea, thiourea, hydroxylamine, guanidine or other amines. When the bath contains an amine it may also contain formaldehyde or a formaldehyde-liberating substance. Particularly good results are obtained with urea and methylated methylolmelamine. The resin concentration in the bath and the amount of liquid taken up by the fabric are so regulated as to incorporate in the fabric 5 to 10% of resin solids by weight of the fabric. The urea combines with the formaldehyde in the bath and with that liberated by the methylolmelamine during the heating of the fabric. In the finished fabric the resin-forming materials are polymerized and combined with the wool.

The following is a process typical of our invention. A light wool fabric was acid dyed with 3% Alizarin Blue SE, Color Index 1053, by a conventional method, and the final rinse adjusted so that the fabric retained about 3% sulfuric acid on the weight of the fabric, as the catalyst for the resin-forming reaction. After being dyed, the fabric was continuously processed at a speed of about 15 yards per minute. It was padded in an impregnating bath containing 6% methylated methylolmelamine solids, 2% urea and 2% alpha trioxymethylene (a source of formaldehyde), by weight of the bath, with a total immersion time of about 10 seconds. The fabric on leaving the bath was squeezed to remove so much of the impregnating solution as to leave in the fabric an amount of the solution equal to about 60% of the dry weight of the fabric. The wet fabric was heated homogeneously throughout from surface to surface by being subjected to the rays of infra-red lamps by which the temperature of the fabric was raised to about 180° F. while retaining about one-third of its water content. The resin-forming materials were changed to a viscous condition so instantly that they did not migrate to the sur-

faces of the fabric but remained homogeneously throughout the fabric.

The fabric, as it advanced, was heated on a tenter and then subjected to the rays of infrared lamps by which its temperature was raised to about 300° F. The methylated methylolmelamine, urea and formaldehyde were polymerized and combined with the wool.

The treated fabric had the same softness, flexibility (hand and feel) and tensile strength as the fabric before treatment. It had no appreciable surface resin which in many treated wool fabrics causes stiffness or a "boardy handle," but the resinous materials were homogeneous from surface to surface of the fabric.

Samples of the treated fabric and similarly dyed, but otherwise untreated, control samples were subjected to standard wool washing tests (CC-T191a, Fed. Spec. for Textiles, Sec. IV, part 5, Par. XIV) and to standard perspiration tests. The treated specimens were found to retain fabric character and dimensional stability after repeated laundering. The shrinkage of the warp, for example, after eight launderings was found to be 0.3%, while the shrinkage of the warp of the control samples after the same eight launderings was found to be 17.5%.

The treated specimens did not bleed in laundering or stain multi-fiber test cloth and after eight standard launderings were found to retain their brilliance and depth of color shade. The controls bled badly, were seriously altered in color after three standard launderings and would be considered unserviceable, from a color standpoint, after five launderings. The treated samples were given a standard alkaline perspiration test and were not altered in shade and did not produce any bleeding on the white test cloth. The controls, however, became streaky, changed in shade and bled badly onto the test cloth.

The tensile strengths of both warp and filling of the treated samples were as good as those of the controls in all cases and in some specimens they were noticeably better.

In our process the urea, or its equivalent, and the methylolmelamine and formaldehyde are polymerized and combined with the wool. Sufficient urea may be included in the impregnating bath to react with all of the formaldehyde liberated from the methylolmelamine during the resin-forming reaction. We may add larger amounts of urea, up to about 50% of the weight of the methylolmelamine, and in this case the bath should include an amount of formaldehyde, or a formaldehyde-liberating substance, sufficient to provide a total of 1 to 2 mols of formaldehyde for each mol of urea at the time of reaction.

We prefer to provide the catalyst as residual acid or acid salt remaining in the fabric from the dyeing operation or supplied by padding with such acid and may use for this purpose inorganic acids such as sulfuric, hydrochloric, or phosphoric or organic acids such as formic, tartaric, maleic or itaconic or their salts. These ways of introducing the catalyst avoid the necessity of including a catalyst as an ingredient in the impregnating bath. The acid should be present in the fabric, when it is heated, in an amount sufficient to provide a pH of about 2 to 5.

The resin-treated wool fabrics disclosed herein are disclosed and claimed in my continuation-in-part application Serial No. 194,942 filed November 9, 1950.

We claim:

1. The method of treating a wool fabric to en-

hance its dimensional stability under laundering conditions while preserving its properties of flexibility, tensile strength and soft hand and feel substantially equal to those of the untreated fabric, which comprises impregnating the fabric with an aqueous solution of 5% to 10% of the weight of the fabric of resin-forming materials comprising a methylolmelamine and formaldehyde, exposing the wet impregnated fabric to infra-red radiation to heat it substantially uniformly from surface to surface and immediately raise its temperature to 140° F. to 212° F. so that sufficient water is almost instantly driven off to leave about one-third of the original water content, thus converting said resin-forming materials to a viscous condition while said solution is maintained uniformly distributed through the whole thickness of the fabric, whereby said materials are immobilized therein against migration to the surfaces of the fabric, and thereafter polymerizing said resin-forming materials to water-insoluble condition by further heating the fabric to a temperature of 212° F. to 300° F.

2. The method of treating a wool fabric to enhance its dimensional stability under laundering conditions while preserving its properties of flexibility, tensile strength and soft hand and feel substantially equal to those of the untreated fabric, which comprises impregnating the fabric with an aqueous solution of 5% to 10% of the weight of the fabric of resin-forming materials comprising a methylolmelamine and formaldehyde, exposing the wet impregnated fabric to infra-red radiation to heat it substantially uniformly from surface to surface and immediately raise its temperature to 180° to 212° F. so that sufficient water is almost instantly driven off to leave about one-third of the original water content, thus converting said resin-forming materials to a viscous condition while said solution is maintained uniformly distributed through the whole thickness of the fabric, whereby said materials are immobilized therein against migration to the surfaces of the fabric and thereafter polymerizing said resin-forming materials to water-insoluble condition by further heating the fabric to a temperature of 212° to 300° F.

3. The method of treating a wool fabric to enhance its dimensional stability under laundering conditions while preserving its properties of flexibility, tensile strength and soft hand and feel substantially equal to those of the untreated fabric, which comprises impregnating the fabric with an aqueous solution of 5% to 10% of the weight of the fabric of resin-forming materials comprising an alkylated methylolmelamine and formaldehyde, exposing the wet impregnated fabric to infra-red radiation to heat it substantially uniformly from surface to surface and immediately raise its temperature to 140° F. to 212° F. so that sufficient water is almost instantly driven off to leave about one-third of the original water content, thus converting said resin-forming materials to a viscous condition while said solution is maintained uniformly distributed through the whole thickness of the fabric, whereby said materials are immobilized therein against migration to the surfaces of the fabric and thereafter polymerizing said resin-forming materials to water-insoluble condition by further heating the fabric to a temperature of 212° to 300° F.

4. The method of treating a wool fabric to enhance its dimensional stability under laundering conditions while preserving its properties of flexibility, tensile strength and soft hand and feel

substantially equal to those of the untreated fabric, which comprises impregnating the fabric with an aqueous solution of 5% to 10% of the weight of the fabric of resin-forming materials comprising an alkylated methylolmelamine, urea and formaldehyde, exposing the wet impregnated fabric to infra-red radiation to heat it substantially uniformly from surface to surface and immediately raise its temperature to 140° F. to 212° F. so that sufficient water is almost instantly driven off to leave about one-third of the original water content, thus converting said resin-forming materials to a viscous condition while said solution is maintained uniformly distributed through the whole thickness of the fabric, whereby said materials are immobilized therein against migration to the surfaces of the fabric and thereafter polymerizing said resin-forming materials to water-insoluble condition by further heating the fabric to a temperature of 212° to 300° F.

5. The method of treating a wool fabric to enhance its dimensional stability under laundering conditions while preserving its properties of flexibility, tensile strength and soft hand and feel substantially equal to those of the untreated fabric, which comprises impregnating the fabric with an aqueous solution of 5% to 10% of the weight of the fabric of resin-forming materials comprising a methylated methylolmelamine, urea and formaldehyde, exposing the wet impregnated fabric to infra-red radiation to heat it substantially uniformly from surface to surface and immediately raise its temperature to 140° F. to 212° F. so that sufficient water is almost instantly driven off to leave about one-third of the original water content, thus converting said resin-forming materials to a viscous condition while said solution is maintained uniformly distributed through the whole thickness of the fabric, whereby said materials are immobilized therein against migration to the surfaces of the fabric and thereafter polymerizing said resin-forming materials to water-

10  
15

20  
25

30

35  
40

insoluble condition by further heating the fabric to a temperature of 212° F. to 300° F.

6. The method of treating a wool fabric to enhance its dimensional stability under laundering conditions while preserving its properties of flexibility, tensile strength and soft hand and feel substantially equal to those of the untreated fabric, which comprises impregnating the fabric with an aqueous solution of 5% to 10% of the weight of the fabric of resin-forming materials comprising a methylated methylolmelamine, urea and formaldehyde, exposing the wet impregnated fabric to infra-red radiation to heat it substantially uniformly from surface to surface, and immediately raise its temperature to 180° F. to 212° F. so that sufficient water is almost instantly driven off to leave about one-third of the original water content, thus converting said resin-forming materials to a viscous condition while said solution is maintained uniformly distributed through the whole thickness of the fabric, whereby said materials are immobilized therein against migration to the surfaces of the fabric, and thereafter polymerizing said resin-forming materials to water-insoluble condition by further heating the fabric to a temperature of 212° F. to 300° F.

JOHN N. DALTON.

WILLIAM B. KAUPIN.

#### REFERENCES CITED

The following references are of record in the file of this patent:

#### UNITED STATES PATENTS

| Number     | Name             | Date          |
|------------|------------------|---------------|
| Re. 22,566 | Johnstone et al. | Nov. 21, 1944 |
| 1,470,990  | Lucas            | Oct. 16, 1923 |
| 1,845,322  | Neuhauß          | Feb. 16, 1932 |
| 2,121,006  | Bener            | June 21, 1938 |
| 2,190,672  | Meharg           | Feb. 20, 1940 |
| 2,248,696  | Cassel           | July 8, 1941  |
| 2,321,938  | Quinn            | June 15, 1943 |